

Feb. 2, 1932.

H. SCOTT

1,843,903

ALLOY

Filed Aug. 11, 1927



INVENTOR

Howard Scott.

BY

*Wesley G. Clegg*  
ATTORNEY

## UNITED STATES PATENT OFFICE

HOWARD SCOTT, OF WILKINSBURG, PENNSYLVANIA, ASSIGNOR TO WESTINGHOUSE ELECTRIC & MANUFACTURING COMPANY, A CORPORATION OF PENNSYLVANIA

## ALLOY

Application filed August 11, 1927. Serial No. 212,202.

My invention relates to alloys and more particularly to alloys having a high coefficient of expansion.

An object of the invention is to provide a metallic alloy having a high coefficient of expansion that is uniform over a wide range of temperatures, the alloy being also adapted to preserve its strength at high temperatures.

Another object of the invention is to provide a metallic alloy, the chief constituents of which are iron, manganese and nickel, that possesses a high coefficient of expansion up to a temperature of 600° C., which makes it particularly useful as an element of a composite bimetallic article made up of two metals of relatively different coefficients of expansion.

A further object of the invention is to provide an alloy which shall have a high coefficient of expansion that is almost linear, and which will, therefore, find special application in thermostats requiring high linear expansion over a wide range of temperature.

In the single figure of the accompanying drawing, the curves show a comparison of one of the improved nickel-iron-manganese alloys containing, in this instance, 10 per cent nickel and 10 per cent manganese, with brass, Monel metal and 23 per cent manganese steel. The ordinates of the curve chart represent unit expansion in thousandths, and the abscissæ represents degrees centigrade.

Brass and Monel metal have commonly been employed for purposes which demand high thermal expansivity. Brass, however, cannot be employed much above normal temperatures, because of its rapid loss of elastic strength with increasing temperatures, which results in permanent deformation.

While the elastic strength of Monel metal is higher than brass, it is still too low for Monel metal to be desirable as an element in a high-temperature bimetal member. Cold rolling partially overcomes this defect, but heating cold rolled metals causes a permanent

loss in strength due to recrystallization, which is greater, the higher the temperature, the longer the exposure at high temperatures, and the greater the cold rolling. The high temperature strength and expansivity of a 23 per cent manganese steel has been found quite satisfactory, but this amount of manganese renders the alloy hard, making it difficult to work, and, furthermore, manganese steel has a low coefficient of expansion at low temperatures, which is sometimes undesirable.

I have found that an alloy composed essentially of iron, nickel and manganese, mixed in such proportions that two and one-half times the amount of manganese plus the amount of nickel in the alloy will not be less than 30 or more than 36 per cent, is easily workable, has a high coefficient of expansion over a wide range of temperatures, and if the manganese and nickel are added in substantially equal proportions, the coefficient of expansion will be substantially linear.

The qualities required in high expansion metal for alloys are (1) high coefficient of expansion throughout the working range, (2) a sufficient elastic strength so that it will not suffer permanent deformation at any required temperature and (3) permanence of its elastic properties. It has been difficult to find a metal or alloy that has all of these characteristics, as metals of high elastic strength are characterized by low expansivity. Pure iron is no exception to this rule, for, if heated gradually, it will be found that iron has a low coefficient of expansion that is almost uniform up to about 900 degrees centigrade, but at this temperature the metal undergoes a change in crystalline structure known as a "transformation point" of the iron. Up to 900 degrees centigrade, the crystalline structure of iron is known as alpha iron. From 900 to 1400 degrees C. pure iron expands uniformly but at a much higher rate than it does at temperatures below 900 degrees C. The

increased coefficient of expansion between the temperatures of 900 and 1400 degrees centigrade is the property of a new crystalline structure known as gamma iron or austenite. The coefficient of expansion of alpha iron is  $10$  to  $15 \times 10^{-6}$  centimeters per centimeter for each degree centigrade, whereas the coefficient of expansion of gamma iron or austenite is substantially  $20$  to  $25 \times 10^{-6}$  centimeters per centimeter for each degree centigrade.

By the addition of suitable proportions of manganese and nickel to iron, the high expansive characteristic of gamma iron can be made available at ordinary temperatures.

I have discovered that the alloy thus provided has the desirable qualities of high elastic strength and a high reversible coefficient of expansion over a long temperature range, combined with excellent workability.

This combination of qualities is not available in either the iron-nickel or iron-manganese system of alloys. An iron base alloy with a high nickel content and without manganese has a high coefficient of expansion,

but this property is not useful because of an irreversible transformation occurring near ordinary temperatures. When the nickel content is sufficiently high to suppress the irreversible transformation, a low coefficient of expansion, similar to that obtained in the well-known alloy invar, occurs at and above ordinary temperatures. The same phenomenon of low expansivity at and near normal

temperatures occurs in high manganese-iron alloys, which have the additional undesirable feature of being workable only with difficulty. However, if manganese and nickel are added to iron in proportions such that the nickel content plus two and one-half times the manganese content are about 32 per cent, the irreversible transformation will not appear and a high coefficient of expansion may be obtained at a temperature ranging from  $-100^{\circ}$  C. to  $600^{\circ}$  centigrade.

The alloy may be produced by the ordinary well known metallurgical processes, such as by melting iron, nickel and manganese together, and it may also contain small percentages of impurities, although carbon should not be present in amounts greater than 0.3 per cent. When a greater amount of carbon than .3 of a per cent is added, however, the expansion characteristics become irreversible. It is, therefore, essential that the amount of carbon should not exceed .3 per cent.

The characteristics of my improved alloy will be more readily understood by referring to the single figure of the drawing, in which brass is represented by curve 5, my manganese-nickel-iron alloy, composed in this instance of 10 per cent manganese and 10 per cent nickel, by curve 6, Monel metal by curve 7, and 23 per cent manganese steel by curve

8. It will be seen from the drawing that while the manganese-nickel-iron alloy does not have quite as high a coefficient of expansion as brass or Monel metal at low temperatures, its coefficient of expansion rapidly increases to the useful high expansion range as the temperature increases. At low temperatures, its rate of expansion is higher and considerably more uniform than 23 per cent manganese steel.

To more clearly exemplify the expansion characteristics of my improved high expansion alloy, the following table showing the coefficients of expansion of an iron-manganese-nickel alloy having the most desirable content of nickel, in comparison with the alloys previously mentioned, is given. In studying the expansion characteristics of the iron-manganese-nickel alloy, it will be remembered that it has greater elastic strength than either brass or Monel metal and is more flexible and easily workable than 23 per cent manganese steel.

*Expansion coefficients at low and high temperatures of high expansion alloys*

| Temperature<br>in degrees<br>centigrade | Coefficient of expansion (unit expansion per $^{\circ}$ C. $\times 10^{-6}$ ) |         |                           |                 | 95  |
|-----------------------------------------|-------------------------------------------------------------------------------|---------|---------------------------|-----------------|-----|
|                                         | Monel                                                                         | Brass   | 10% Mn<br>10% Ni<br>steel | 23% Mn<br>steel |     |
| -150                                    | 12.1                                                                          | 18.8    | 8.3                       | 8.3             |     |
| -100                                    | 12.9                                                                          | 19.2    | 11.8                      | 8.5             |     |
| -50                                     | 13.6                                                                          | 19.6    | 16.3                      | 9.0             |     |
| 0                                       | 14.3                                                                          | 20.1    | 18.2                      | 9.7             |     |
| +50                                     | 15.0                                                                          | 20.5    | 18.8                      | 11.5            |     |
| 100                                     | 15.4                                                                          | 21.0    | 19.5                      | 14.5            | 100 |
| 150                                     | 15.7                                                                          | 21.4    | 20.2                      | 17.5            |     |
| 200                                     | 16.0                                                                          | 21.9    | 20.8                      | 19.4            |     |
| 250                                     | 16.4                                                                          | 22.3    | 21.5                      | 20.6            |     |
| 300                                     | 16.7                                                                          | 22.6    | 22.2                      | 21.6            |     |
| 350                                     | 17.0                                                                          | Softens | 22.8                      | 22.6            |     |
| 400                                     | Softens                                                                       |         | 23.5                      | 23.6            |     |
| 450                                     |                                                                               |         | 24.2                      | 24.5            |     |
| 500                                     |                                                                               |         | 24.8                      | 25.5            | 105 |

It is to be clearly understood that while curve 5, and the tables, show the coefficient of expansion of an iron alloy containing 10% manganese and 10% nickel, these proportions may be varied and a satisfactory alloy produced when nickel is present in amounts ranging from 1 to 34 per cent, and the manganese in amounts ranging from 12 to 1 per cent, it only being necessary that the manganese and nickel be added in such proportions that two and one half times the manganese, plus the nickel, will not be less than 30, nor more than 36 per cent.

It is recognized that the coefficient of expansion of alloys vary in accordance with the impurities present and the proportion of the ingredients. In comparing my improved alloy with Monel metal, brass and 23% manganese steel, it will therefore be understood that the impurities and ingredients of these alloys are present in such proportions that they will have the coefficient of expansion specified in the above table.

Various modifications may be made in prac-

ticing my invention without departing from the spirit and scope thereof. I desire, therefore, that only such limitations shall be placed thereon as are imposed by the prior art and the appended claims.

5 I claim as my invention:

1. An alloy containing not more than .3% carbon and comprising about 80% of iron, about 10% of nickel and about 10% of manganese, said alloy having a coefficient of expansion approximately equal to that of brass.

10 2. An alloy having a high reversible temperature coefficient of expansion comprising 5 to 30% nickel, manganese in amounts ranging from 12 to 2% in accordance with the amount of nickel present and the remainder iron and minor impurities, said alloy containing not more than .3% carbon and the amount of nickel plus two and one-half times the manganese being not less than 30% nor more than 36% of the alloy.

15 3. An alloy having a high reversible temperature coefficient of expansion and comprising from 6 to 28% nickel, manganese in amounts ranging from 11 to 3% in accordance with the amount of nickel present and the remainder iron and minor impurities, said alloy containing not more than .3% carbon and the amount of nickel plus two and one-half times the manganese being not less than 30% nor more than 36% of the alloy.

20 4. An alloy having a high reversible temperature coefficient of expansion and comprising from 8 to 24% nickel, manganese in amounts ranging from 10 to 4% in accordance with the amount of nickel present and the remainder iron and minor impurities, said alloy containing not more than .3% carbon and the amount of nickel plus two and one-half times the manganese being not less than 30% nor more than 36% of the alloy.

25 5. An alloy having a high reversible temperature coefficient of expansion and comprising from 10 to 20% nickel, manganese in amounts ranging from 10 to 6% in accordance with the amount of nickel present and the remainder iron and minor impurities, said alloy containing not more than .3% carbon and the amount of nickel plus two and one-half times the manganese being not less than 30% nor more than 36% of the alloy.

30 6. An alloy having a high reversible temperature coefficient of expansion and comprising from 10 to 16% nickel, manganese in amounts ranging from 10 to 7% in accordance with the amount of nickel present and the remainder iron and minor impurities, said alloy containing not more than .3% carbon and the amount of nickel plus two and one-half times the manganese plus two and one-half times the manganese being not less than 30% nor more than 36% of the alloy.

35 7. An alloy having a high reversible temperature coefficient of expansion and com-

prising from 10 to 14% nickel, manganese in amounts ranging from 10 to 8%, in accordance with the amount of nickel present and the remainder iron and minor impurities, said alloy containing not more than .3% carbon and the amount of nickel plus two and one-half times the manganese being not less than 30% nor more than 36% of the alloy.

40 In testimony whereof, I have hereunto subscribed my name this 3rd day of August, 1927.

HOWARD SCOTT.

80

85

90

95

100

105

110

115

120

125

130